

1

2,944,385

## STABLE MONOPROPELLANTS

Emory E. Toops, Jr., Terre Haute, Ind., assignor to Commercial Solvents Corporation, Terre Haute, Ind., a corporation of Maryland

No Drawing. Filed May 19, 1958, Ser. No. 735,920

5 Claims. (Cl. 60—35.4)

My invention relates to new propellants for reaction motors, and more particularly, to propellant mixtures of lithium chlorate in ammonia.

The missile industry has been unable to formulate a stable, non-corrosive, relatively insensitive monopropellant which can be easily stored and handled without endangering the life and health of personnel working in the area. Compounds such as ethylene oxide nitromethane, tetranitromethane, propyl nitrate, etc. have found some use as monopropellants in reaction motors. There has been no wide acceptance of these materials as monopropellants, due to the extreme shock sensitivity or reactivity inherent in these products.

I have now discovered that solutions of lithium chlorate in ammonia are excellent monopropellants and fuels. As the oxygen balance of my new lithium chlorate-ammonia solutions can be varied over a wide range, my compositions find a variety of uses in the propellant field. Some of my new compositions, having a high ratio of reducing potentials to oxidizing potentials, are useful as fuels for air-breathing engines, such as pulse jets and ramjets, and as fuels for bipropellant reaction motor systems; while my solutions having approximately equal ratios of oxidizing potentials to reducing potentials are excellent monopropellants in that they are thermally stable and relatively insensitive to shock resulting from induced pressures or impact.

It is known that ammonia will dissolve many oxidant salts. It is also known that most oxidant salts are too insoluble in ammonia to form mixtures suitable for use as monopropellants. No ammonia-oxidant salt mixtures are known which have oxygen balances such that the systems could be used as liquid monopropellants. Known mixtures are exemplified by Divers solution, which is so difficult to burn that it cannot be used as a monopropellant. Unexpectedly, I have found that ammonia-lithium chlorate mixtures, having suitable oxygen balances, have very rapid burning rates and low ignition temperatures when compared with other ammonia-oxidant salt solutions, and as a result, are excellent monopropellants.

I have also determined that up to one quarter mole of water can be added to my propellant mixtures per mole of ammonia. The addition of desired amounts of water allows me to regulate the combustion chamber temperatures to some extent, to lower viscosity, and to modify burning characteristics.

Various other inert additives may be added to my mixtures as needed, up to about 20% by weight. Such additives must be inert to the extent that they do not react with lithium chlorate, ammonia or other additives at ordinary storage temperatures and pressures in such a manner as to reduce materially the desired explosive or propellant properties of the mixtures. The inert additives may be introduced into my mixtures to sensitize or desensitize the compositions, to add oxidizing or reducing potentials to the compositions, to catalyze the burn-

2

ing rate of the mixtures, to make the mixtures hypergolic with strong oxidants, to depress the freezing points of the mixture, to lower the average molecular weight of the exhaust gases or to reduce the burning temperatures of the mixtures. Additives which act as fuels in my mixtures include hydrazine; metals such as aluminum and magnesium; boranes; alcohols such as methanol and ethanol; etc. Additives which I have found useful in adding oxidizing potentials to my compositions include nitrosyl fluoborate, monomethylamine nitrate, monomethylamine perchlorate, etc. Water may be added to my composition to increase the volume of the combustion products formed and to decrease the burning temperatures of my compositions.

Oxidants which may be utilized with my fuel mixtures in bipropellant systems are any of the commonly used oxidants, such as liquid oxygen, red and white fuming nitric acid, dinitrogen tetroxide, etc.

My new compositions have specific impulses of about 210, on the order of some commonly used liquid bipropellant systems, while being relatively economical to prepare. As my propellant solutions have relatively high densities, on the order of 1.3 or more, they have impulse densities in excess of 280.

My new lithium chlorate-ammonia mixtures are relatively non-corrosive to cold rolled steel and aluminum and are non-reactive with rubber, Teflon, polyethylene, etc.

The compositions of my invention have very low vapor pressures, on the order of about 5 pounds at 25° C.

The compositions of my invention can contain from about 2 to about 3 moles of ammonia per mole of lithium chlorate. A solution containing two moles of ammonia and one mole of lithium chlorate is in exact oxygen balance. However, slightly better performance is obtained when the propellant solution is slightly fuel-rich.

My new compositions are prepared by passing anhydrous ammonia into the solid lithium chlorate salt. I prefer to prepare my compositions at temperatures below the boiling point of anhydrous ammonia, due to ease of handling.

My compositions are easily adapted to a variety of uses in the propellant field. My compositions having reducing potentials in the range of 5 to 15% in excess of the oxidizing potentials are excellent monopropellants. Solutions that are very fuel-rich, containing from 20 to 40% excess reducing potentials are useful as bipropellant fuels in rockets or fuels for ramjets, etc.

To utilize the propellant solutions of my invention, I introduce them, at a desired rate, into a reaction chamber containing a suitable igniter, such as a starting squib or a white hot platinum grid, to initiate combustion. Once combustion has begun, the heating element can be removed, or, in the case of platinum heaters, can remain within the reaction motor to catalyze the burning rate of the propellant.

As previously stated, compositions containing from 20 to 40% excess reducing potentials are useful as fuels for reaction motors such as ramjets and as fuels for bipropellant rocket systems. The use of such mixtures as fuels for bipropellant systems means that less oxidant is required as the high specific gravity fuel carries considerable amounts of oxygen.

When my compositions are used in air-breathing engines, such as ramjets or pulse jets, principles of operation which apply are similar to those applicable to present day engines employing ordinary hydrocarbon fuels. In all of these engines the oxygen in the air is mixed with the fuel so that the fuel-air ratio is approximately stoichiometric. In this way, complete burning and efficient operation of the engine is assured. For example,

when a 50% lithium chloride, 50 wt. percent ammonia mixture is used as a ramjet engine fuel, a ratio of 1.9:1 air to fuel by weight is desired. This fuel produces about 1930 B.t.u. per pound of air used while standard hydrocarbon fuels produce only about 1200-1300 B.t.u. per pound of air. During or after combustion of my fuels in the combustion chambers of the reaction engines large amounts of excess air are passed through the engines in order that the combustion chamber walls may be maintained at desired temperatures.

The following table discloses the physical properties of a representative propellant solution of my invention containing one mole of lithium chloride to two moles of ammonia. As previously stated, this composition is in oxygen balance.

|                                       |      |
|---------------------------------------|------|
| Density, 25° C                        | 1.35 |
| Specific impulse at 300 p.s.i.a., sec | 210  |
| Impulse density, sec                  | 283  |
| Viscosity, centipoises at:            |      |
| 25° C                                 | 65   |
| 20° C                                 | 79   |
| 10° C                                 | 122  |
| 0° C                                  | 198  |
| -10° C                                | 343  |
| Vapor pressure mm.abs. at 25° C       | 220  |

The following table sets out the solubility of various amounts of lithium chloride in ammonia.

#### SOLUBILITY OF ANHYDROUS LITHIUM CHLORATE IN ANHYDROUS AMMONIA

| Percent wt.<br>lithium<br>chlorate | Percent<br>wt. am-<br>monia | mole ratio,<br>ammonia;<br>chlorate | observations                                              |
|------------------------------------|-----------------------------|-------------------------------------|-----------------------------------------------------------|
| 84                                 | 16                          | 1:1                                 | undissolved chlorate fluid suspension.                    |
| 78                                 | 22                          | 1.5:1                               | some chlorate still undis-<br>solved.                     |
| 72.6                               | 27.4                        | 2:1                                 | few specks chlorate remain-<br>ing, solution quite fluid. |
| 67.6                               | 32.4                        | 2.5:1                               | all chlorate dissolved.                                   |

The following specific examples more fully illustrate my invention, but it is not intended that my invention be limited to the processes, reaction motors or fuels described therein, but rather it is intended that all equivalents obvious to those skilled in the art be included within the scope of my invention as claimed.

#### Example I

To test one of my compositions as a monopropellant 0.18 pounds per second of a 2:1 molar ratio of monomethylamine to lithium chloride was injected into a small rocket thrust chamber through four converging injection nozzles. This propellant burns well and has a specific impulse of 209 seconds.

#### Example II

To test one of my propellant compositions in a bipropellant system a small thrust chamber made up of available 1" stainless steel pipe and stainless steel pipe

5 fittings was prepared. The fuel injection nozzle was made from a pipe plug. An orifice diameter of 0.040" was drilled in the pipe plug and the needle valve assembly was seated in and welded onto the plug. For ease of 10 repair a 1" union was used to attach the nozzle to the 4" pipe which comprises the burning chamber. An oxygen inlet tube and a Bourdon-type pressure gauge with a range of 0-600 p.s.i. were attached to the burning chamber through the plug. A reducing coupling was utilized 15 as the motor nozzle. A reaction mixture having a molar ratio of 3:1 ammonia to lithium chloride was introduced into the thrust chamber through the injector nozzle at a rate of 0.2 cu. ft. per minute. An approximately stoichiometrically equal amount of gaseous oxygen was also introduced into the thrust chamber. Ignition was initiated by preheating the chamber to 625° C. The fuel burned well with good thrust.

This application is a continuation-in-part of my U.S. patent application Serial No. 704,361 filed December 23, 20 1957 now abandoned.

Now having described my invention what I claim is:

1. Monopropellant mixtures consisting essentially of lithium chloride-ammonia mixtures having a molar ratio of lithium chloride to ammonia ranging from about 1:2 to about 1:3, and an inert additive selected from the group consisting of lower alkyl alcohols, water, monomethylamine nitrate and monomethylamine perchlorate.

2. Monopropellant mixtures consisting essentially of lithium chloride-ammonia mixtures containing a ratio of 30 1 mole of lithium chloride to about 3 moles of ammonia and up to 0.25 mole of water per mole of ammonia.

3. In a process for producing thrust in a reaction motor which comprises burning, in a reaction motor, mixtures having a molar ratio of lithium chloride to ammonia ranging from about 1:2 to about 1:3.

4. The process for producing thrust in a monopropellant burning reaction motor which comprises burning, in a monopropellant burning reaction motor, a mixture of lithium chloride in ammonia, said mixture having a 40 molar ratio of 2.5:1 ammonia to lithium chloride.

5. The process for producing thrust in a bipropellant burning reaction motor which comprises burning, in a bipropellant burning reaction motor, mixtures having a molar ratio of lithium chloride to ammonia ranging from 45 about 1:2 to about 1:3 and a bipropellant oxidant selected from the group consisting of liquid oxygen, red and white fuming nitric acid and dinitrogen tetroxide.

#### References Cited in the file of this patent

#### UNITED STATES PATENTS

|           |                |               |
|-----------|----------------|---------------|
| 1,506,323 | O'Neill        | Aug. 26, 1924 |
| 2,393,594 | Davis          | Jan. 29, 1946 |
| 2,811,431 | Zwickly et al. | Oct. 29, 1957 |

#### OTHER REFERENCES

Ephraim: "Berichte der Deutschen Chemischen Gesellschaft," vol. 52, page 240.

Zeitschrift fur das gesamte Schiess and Sprengstoff-  
60 wesen, Apr. 1926, vol. 21, Nov. 4, pages 49-52.